

**1**

3,573,903

**DUCTILE HIGH TEMPERATURE TUNGSTEN-RHENIUM ALLOY AND PROCESS FOR MAKING SAME**

Eugene J. Delgrosso, Wallingford, Conn., assignor to United Aircraft Corporation, East Hartford, Conn.  
No Drawing. Filed July 21, 1964, Ser. No. 385,101  
Int. Cl. C22c 27/00

U.S. Cl. 75—176

11 Claims

**ABSTRACT OF THE DISCLOSURE**

A novel ductile high-temperature tungsten-base alloy containing 3 to 20% rhenium and .05 to 3.0% yttrium or mixtures of yttrium and cerium is made by compacting powders of the ingredient elements, heating the compact at an intermediate temperature well below the compact's sintering temperature in a hydrogen atmosphere to effect removal of interstitials, and then sintering the compact in a dynamic vacuum.

This invention relates to novel tungsten-base alloys having tungsten as their principal component and to a method for making such alloys.

More particularly, this invention relates to novel tungsten-rhenium alloys containing small amounts of yttrium or yttrium and cerium. Such alloys are ductile at room temperature and are capable of being formed into tube, sheet and other configurations by conventional fabrication methods.

These alloys are created by compacting powders of the ingredient elements, heating the powdered compact at an intermediate temperature well below the compact's sintering temperature in a hydrogen atmosphere to effect removal of interstitials, and then sintering the compact in a dynamic vacuum.

Tungsten-rhenium alloys have been well known for many years. The principal use of such alloys has been in thermocouples for measuring unusually high temperatures. A typical tungsten-rhenium alloy for use in such thermocouples is tungsten-30% rhenium by weight. Normally, such thermocouples comprise one leg consisting of W-30% Re by weight (W-30Re) and a second leg consisting of pure tungsten or a low rhenium content alloy such as W-3 to 6% Re by weight.

Tungsten-rhenium thermocouples are used to control temperatures in high-temperature vacuum furnaces, rupture rigs and reactors. They are generally considered to be the best commercially available high-temperature thermocouples.

Rhenium has also been used as a solid solution softener of tungsten. Because of its high melting point and ability to retain high strength at high temperatures, tungsten potentially is one of the best alloy bases for high-temperature structural uses in nuclear fuel containment vessels, thermionic emitters, reactors, rockets and electrical and electronic devices.

Great problems have been encountered, however, in attempting to use tungsten in forming structural parts because of its brittleness at room temperature and temperatures at which it can be conveniently worked using conventional fabrication methods. Although pure tungsten exhibits ductility in the lower temperature ranges, tungsten has great affinity for oxygen and nitrogen, which leads to its rapid embrittlement whenever it is exposed to air.

In amounts up to about 50% by weight rhenium forms a solid solution with tungsten. It has been known for some years that rhenium in amounts of 25% or more by weight, when added to tungsten in solid solution, counteracts the embrittling effect of oxygen and nitrogen inter-

**2**

stitials in the tungsten and promotes ductility in the resulting alloy. It is believed that rhenium causes the oxygen and nitrogen in the grain boundaries to form discontinuous globules in place of the brittle continuous grain boundary envelope-type films normally formed by oxygen and nitrogen as interstitials in pure tungsten. These rhenium induced globules permit slippage between grain boundaries and result in an alloy exhibiting ductility at temperatures down to and including room temperature.

In recent years this ductility improving characteristic of rhenium has resulted in development of semicommercial W-Re alloys that retain ductility at room temperature. Such alloys, however, must contain at least 25% rhenium by weight to effectively counteract the embrittling oxygen and nitrogen interstitials. Semicommercial W-25Re alloys has been used for making both wire and thermocouples. Potentially, it is also a candidate for the manufacture of high-temperature structural parts.

Unfortunately, however, rhenium is a very rare metal. Its cost currently runs as high as \$1500 per pound. Since the semicommercial alloy requires at least 25% rhenium by weight in solid solution with tungsten to achieve room temperature ductility, the cost of suitable tungsten-rhenium alloys for structural materials is almost prohibitive.

It is accordingly a primary object of this invention to provide tungsten-rhenium alloys and a method for making them in which the rhenium content can be reduced to amounts of as little as 3% rhenium by weight without sacrificing room temperature ductility.

Another object of this invention is to provide a novel and improved tungsten-rhenium alloy containing small amounts of rhenium and even smaller amounts of yttrium or a mixture of yttrium and cerium that exhibits room temperature ductility and permits fabrication of structural parts by conventional methods at moderate fabrication temperatures. This invention thus achieves tungsten alloys containing as little as 3% by weight rhenium that can be fabricated into tube and sheet type structural parts by conventional fabrication methods.

It is another object of this invention to provide a new and improved process for producing a ductile tungsten-rhenium alloy containing small amounts of rhenium that simultaneously achieves purification of the tungsten base and formation of a ductile tungsten-rhenium alloy.

Yet another object of this invention is to provide a new and improved tungsten-rhenium alloy and process for making it that yields an alloy having distinctly improved resistance to corrosion at high temperatures. The alloys of this invention thus have exceptionally improved resistance to corrosion by the alkali metals, particularly liquid lithium, when used as structural tubing in reactors.

A further object of this invention is to provide a new and improved tungsten-rhenium alloy containing small amounts of rhenium and even smaller amounts of yttrium in which yttrium promotes thermionic properties in the alloy and achieves an alloy having enhanced value as a thermionic emitter or thermionic converter over conventional tungsten-rhenium alloys.

The high amounts of rhenium required in prior art tungsten-rhenium alloys to achieve ductility degrade the overall strength of such alloys. It is thus an important object of the present invention to provide a tungsten-rhenium alloy that attains ductility with the use of much less rhenium than is required in prior art alloys. The ductile tungsten-base alloys of this invention accordingly have appreciably greater strength and are must less expensive than similar prior art alloys.

Additional objects and advantages will be set forth in part in the description that follows, and in part will be obvious from the description, or may be learned by practice of the invention, the objects and advantages being realized and attained by means of the compositions,

methods and processes particularly pointed out in the appended claims.

To achieve the foregoing objects in accordance with its purpose, this invention includes a high-temperature ductile alloy consisting essentially of tungsten as the principal component, from 3 to 20% by weight of rhenium, and from .05 to 3% by weight of a metal additive selected from the group consisting of yttrium and mixtures of yttrium and cerium.

The invention further comprehends a process of producing a high-temperature ductile alloy consisting essentially of tungsten as the principal component, from 3 to 20% by weight of rhenium, and from .05 to 3% by weight of a metal additive selected from the group consisting of yttrium and mixtures of yttrium and cerium. The process comprises the steps of: compacting a mixture of finely divided powders consisting essentially of from 3 to 20% by weight of rhenium, .05 to 3% by weight of a metal additive selected from the group consisting of yttrium and mixtures of yttrium and cerium and the balance essentially tungsten, heating the resultant compact in a hydrogen atmosphere at a temperature of from 1400 to 2700° F. for a time period sufficient to achieve outgassing of a substantial portion of oxygen and nitrogen interstitials and to impart a density of from 55 to 75% in the compact, sintering the compact in a dynamic vacuum at a temperature of from 3600 to 4200° F. for a time period sufficient to achieve from 85 to 98% density in the compact, thereby creating a ductile tungsten-base alloy having high strength at high temperatures and fabricability at low and moderate temperatures.

For convenience, the first heating step is termed a "presintering" step and the second heating step is termed a "densifying" or "sintering" step.

In a preferred form, the invention also includes within its scope a ductile high-temperature alloy consisting essentially of tungsten as the principal component, from 5 to 15% by weight of rhenium, and from .05 to 3% by weight of a metal additive selected from the group consisting of yttrium and mixtures of yttrium and cerium.

When a mixture of yttrium and cerium is used, the ratio by weight of yttrium to cerium should be from 1:2 to 2:1. A preferred ratio is 1:1. When the mixture is cerium rich, the compact should be heated up more slowly during the presintering step than when the mixture is yttrium rich.

The tungsten, rhenium, yttrium and cerium powders used to produce the alloys of this invention should be of the highest purity practically attainable and usually have a size range of less than 300 mesh (48 microns) although coarser particles, ranging in size from about 100 to 300 mesh (147 to 48 microns) may also be used. Especially good results are obtained when the size range of the powders is less than 400 mesh (38 microns), or between about 0 to 38 microns and preferably between about 0 to 10 microns. In general, it can be said that the finer the particles, the better the alloy compact produced. The mesh sizes reported are Tyler standard.

There has been a long felt need for achieving a ductile tungsten alloy that would be capable of being formed into structural parts such as tube and sheet at moderate working temperatures and that would not require large amounts of rare and expensive rhenium to impart desired ductility. This invention achieved the unexpected new and useful result of making possible a dramatic reduction in rhenium content of tungsten-rhenium alloys and yet still attains the desired room-temperature ductility by the addition of small amounts of yttrium or yttrium and cerium to the charge used to produce the alloy and by controlled process steps used in forming the alloy.

In the process of producing the alloy the yttrium or yttrium and cerium function to eliminate from the tungsten a major proportion of its oxygen and nitrogen interstitials. The removal of these interstitials in turn makes it possible to achieve desired ductility in the alloy with

much smaller amounts of rhenium than would otherwise be required. With the tungsten base freed of most of its interstitials, the small proportion of rhenium used in the alloys of this invention is sufficient to counteract the embrittling effect of any remaining interstitials.

The yttrium content of the alloy provides an additional unexpected new and useful result in reducing the susceptibility of the alloy to corrosion attack by liquid alkali metals, particularly lithium, when used as structural members for reactors or nuclear containment vessels. Yttrium getters interstitial oxygen and forms oxides more stable than lithium oxide; this prevents leaching of oxygen by lithium (or other alkali metals) from less stable rhenium oxides.

The tungsten-rhenium alloy resulting from the process of this invention possesses high ductility and can be readily formed into structural components, such as tubing or sheet, at room or moderate working temperatures. Since substantial amounts (usually about one-half or more by weight) of the yttrium, or yttrium and cerium, originally present as part of the alloy charge may be evolved during the process as vapor phase compounds with oxygen and nitrogen, it sometimes occurs that only minor amounts of yttrium and cerium will be found in the final product. Cerium, partly because of its lower melting point, is particularly susceptible to loss in vapor phase during the presintering and sintering steps.

Accordingly, the charge for producing the alloys of this invention should contain from 1 to 5% by weight of yttrium or a mixture of yttrium and cerium to yield an alloy product containing from .05 to 3% by weight of yttrium or a mixture of yttrium and cerium.

In carrying out the process of this invention, the ingredient elements in the form of metal powders are mixed and compacted in an inert atmosphere. Typically, this can be accomplished in a dry box that is evacuated and back filled with argon, preferably to a little below atmospheric pressure. The powders are then compacted in the inert atmosphere, preferably at a pressure of from 25 to 60 TSI.

The pressed compacts are placed in a protective carrying container and transferred to a high-temperature resistance furnace. The presintering step is carried out in this furnace in which the compacted powders of the alloys are exposed to a high purity hydrogen atmosphere at from 1400 to 2700° F. for a time period sufficient to evolve a major proportion of the various gaseous interstitials in the compact either directly as occluded or adsorbed gases or as vapor phase compounds with yttrium or yttrium and cerium. Preferably, the furnace is operated at about 2200° F. and the desired amount of outgassing can be accomplished in about 2 hours. It is important, however, that the furnace be raised slowly to temperature, since this promotes the release of occluded or adsorbed gases and evolution of vapor phase oxides and nitrides of yttrium and cerium at a steady rate, avoids cracking and fracturing of the compact, and maintains porosity permitting continuous evolution of gases.

In this presintering step the compact achieves a green density of from 55 to 75%, preferably 60 to 70%. The presintering thus gives body to the compact and holds it in its compacted shape. Most of the outgassing of interstitials occurs during this presintering step and improves the results obtained in the densifying step which follows.

Both yttrium and cerium perform gettering functions in the presintering step, since they readily tend to form volatile compounds with oxygen and nitrogen and exhibit a preferential affinity for the oxygen and nitrogen present as interstitials in the tungsten. This results in simultaneous purification and improvement of ductility in the resultant alloy.

Cerium has a lower melting point than yttrium and cerium oxide is volatile at a lower temperature than yttrium oxide. Accordingly, when cerium and yttrium are used together as components of the alloy, the com-

pact during the presintering step may be heated to the melting point of cerium or about 1460° F. and held at that temperature for a time period sufficient to remove quantities of oxygen and nitrogen as vapor phase compounds with cerium, and the temperature can then be slowly increased toward the melting point of yttrium (about 2700° F.), preferably to about 2200° F., to promote evolution of oxygen and nitrogen as vapor phase compounds with yttrium.

In accordance with the invention, residual yttrium remaining in the alloy after sintering improves the overall corrosion resistance of the alloy by its gettering of oxygen to form stable yttrium oxides.

Upon completion of the presintering step the compact is transferred to a vacuum atmosphere furnace capable of maintaining a dynamic vacuum. The compact is then slowly heated to a temperature of from 3600 to 4200° F. with the pumps on and held at that temperature for a time period sufficient to achieve 85 to 98% density in the compact. Generally, this will be from about 1 to 4 hours.

During sintering in the vacuum atmosphere the pressure may rise to about 1000 microns due to continued outgassing of occluded and adsorbed gases and evolution of vapor phase compounds of yttrium and cerium with oxygen and nitrogen. As the sintering step nears completion, the vacuum will be observed to fall back to a pressure of from 10 to 1 microns. When the pressure has dropped off to about 10 microns or less, this is an indication that densifying or sintering has neared or reached completion. At this point the heat may be shut off and the furnace allowed to cool to ambient temperature, when the compact is removed.

The resultant alloy compacts of this process exhibit good warm or cold workability or fabricability and can be treated in much the same manner as the semicommercial W-30Re alloys, even though they may contain as little as 3% by weight of rhenium. For example, the alloys of this invention can be cold or warm swaged or cold or warm forged and then rolled hot or cold.

In accordance with the invention, the additions of yttrium or yttrium and cerium are used to remove almost all of the interstitials from tungsten. Most of the compositional constituents that contribute to the embrittlement of tungsten are eliminated and the embrittling effects of the remaining interstitials are overcome with a much smaller amount of rhenium than has been required with prior tungsten-rhenium alloys.

In this way ductile tungsten alloys can be created using small amounts of rhenium to achieve a stronger and much less expensive high-temperature tungsten-base alloy than has heretofore been possible. Moreover, such ductile tungsten-base alloys can be fabricated at low temperatures without the necessity of resorting to expensive, elaborate and time-consuming preparation processes necessary for high-temperature fabrication of normally brittle tungsten-base alloys, such as sheathing, canning, or sheltering in an inert atmosphere.

For a clearer understanding of the invention, specific examples are set forth below. These examples are merely illustrative and are not to be understood as in any way limiting the scope and underlying principles of the invention.

#### EXAMPLE 1

An intimate mixture of high purity metallic powders of the following composition was carefully prepared in a dry box under an argon atmosphere by milling or V blending:

94 grams of tungsten powder (−300 mesh or finer),  
5 grams of rhenium powder (−300 mesh or finer),  
1 gram of yttrium powder (−300 mesh or finer).

The blended powders were then pressed in a 1 inch diameter breakaway type die at 50 TSI. The compact was next inverted and repressed in the same manner. The blending

and compacting were all performed in an argon atmosphere to avoid atmospheric contamination.

The pressed compact was placed in a high-temperature resistance furnace for presintering. The furnace was evacuated and backfilled with high purity hydrogen to a slight positive pressure. It was then slowly heated to promote outgassing of occluded and adsorbed gases from the surfaces of the particles forming the compact and outgassing of vapor phase compounds of yttrium with interstitials in the constituent elements of the compact.

The temperature in this presintering furnace was slowly raised to 2200° F. and held there for 2 hours. At the end of 2 hours the furnace was allowed to cool to room temperature and the compact was removed. By this presintering step the compact achieved a density of about 65%.

The compact was next placed in a high-temperature vacuum resistance furnace for the densifying step. In this step the temperature was again slowly raised with the pumps on to about 4000° F. and was held at that temperature for about 3 hours. During this step the pressure in the furnace rose to about 1000 microns and then slowly fell back to about 10 microns.

When the pressure reached 10 microns at the end of about 3 hours, the furnace was turned off and allowed to cool to room temperature and the compact withdrawn. The rise in pressure within the dynamic vacuum furnace indicated that there was a continuous evolution of gases from the compact including vapor phase compounds of yttrium with oxygen and nitrogen.

Upon removal from the furnace the compact was found to have achieved a density of about 95%. It was then warm swaged at about 1300° F., with reduction of about 15% per pass. Intermediate anneals at 3000° F. were given as required to avoid cracking, and in this manner the compact was reduced from 1 inch to 1/4 inch diameter. This 1/4 inch rod was then cold swaged at room temperature with reductions of about 10% per pass and an intermediate anneal was given after each pass. The resultant wire was free of slivering and exhibited room temperature ductility.

By contrast, wire produced from W-5Re alloy having no yttrium in the charge from which the alloy was produced silvered badly evidencing embrittlement. Also, grain boundary hardness of the alloy of this example was only one half that of a W-5Re alloy without yttrium.

If warm working is not desired, the alloy of this example can be cold worked directly in the same manner as described for the warm working. This fabrication at room temperature can be accomplished easily and without the formation of injurious cracks, slivers or other evidence of embrittlement. It is apparent from the attributes exhibited that the alloy of this example retains significant ductility at room temperature.

The resultant alloy had the following composition in percent by weight:

|          |      |
|----------|------|
| Tungsten | 94.5 |
| Rhenium  | 5    |
| Yttrium  | 0.5  |

Significantly, about one-half the original charged weight of yttrium was lost in the course of forming the alloy. This yttrium loss is accounted for by the formation and pumping off of vapor phase compounds of yttrium with interstitial oxygen and nitrogen.

#### EXAMPLE 2

A compact was prepared as in Example 1 using an intimate mixture of high purity metallic powders having the following composition:

89 grams of tungsten powder (−300 mesh or finer),  
10 grams of rhenium powder (−300 mesh or finer),  
1 gram of yttrium powder (−300 mesh or finer).

This yielded an alloy of the following composition in percent by weight:

|          |      |
|----------|------|
| Tungsten | 89.5 |
| Rhenium  | 10   |
| Yttrium  | 0.5  |

Results similar to Example 1 were obtained.

#### EXAMPLE 3

An alloy having the following composition in percent by weight was prepared as in Example 1:

|          |      |
|----------|------|
| Tungsten | 84.5 |
| Rhenium  | 15   |
| Yttrium  | 0.5  |

Results similar to Example 1 were obtained.

#### EXAMPLE 4

An alloy having the following composition in percent by weight as in Example 1 was prepared:

|          |      |
|----------|------|
| Tungsten | 79.5 |
| Rhenium  | 20   |
| Yttrium  | 0.5  |

Results similar to those of Example 1 were obtained.

#### EXAMPLE 5

A mixture of high purity metallic powders of the following composition was prepared:

93 grams of tungsten powder (-300 mesh or finer),  
5 grams of rhenium powder (-300 mesh or finer),  
1 gram of yttrium powder (-300 mesh or finer),  
1 gram of cerium powder (-300 mesh or finer).

An alloy was prepared from this composition as set forth in Example 1. This alloy had the following composition percent by weight:

|          |      |
|----------|------|
| Tungsten | 94.2 |
| Rhenium  | 5    |
| Yttrium  | 0.5  |
| Cerium   | 0.5  |

Results similar to those of Example 1 were obtained.

#### EXAMPLES 6-8

The following additional alloys were prepared as in Example 1. Compositions are expressed in terms of percent by weight:

#### EXAMPLE 6

|          |     |
|----------|-----|
| Tungsten | 89  |
| Rhenium  | 10  |
| Yttrium  | 0.5 |
| Cerium   | 0.5 |

#### EXAMPLE 7

|          |     |
|----------|-----|
| Tungsten | 84  |
| Rhenium  | 15  |
| Yttrium  | 0.5 |
| Cerium   | 0.5 |

#### EXAMPLE 8

|          |     |
|----------|-----|
| Tungsten | 79  |
| Rhenium  | 20  |
| Yttrium  | 0.5 |
| Cerium   | 0.5 |

Results similar to those of Example 1 were obtained with each of these alloys exhibiting room temperature ductility and fabricability.

#### EXAMPLE 9

A mixture of high purity metallic powders of the following composition was prepared:

93 grams of tungsten powder (-300 mesh or finer),  
5 grams of rhenium powder (-300 mesh or finer),  
2 grams of yttrium powder (-300 mesh or finer).

An alloy was prepared from this composition as set forth in Example 1. This alloy had the following composition in percent by weight:

|          |    |
|----------|----|
| Tungsten | 94 |
| Rhenium  | 5  |
| Yttrium  | 1  |

Results similar to those of Example 1 were obtained.

#### EXAMPLES 10-12

The following additional alloys were prepared as in Example 1. Compositions are expressed in terms of percent by weight:

#### EXAMPLE 10

|          |    |
|----------|----|
| Tungsten | 89 |
| Rhenium  | 10 |
| Yttrium  | 1  |

#### EXAMPLE 11

|          |    |
|----------|----|
| Tungsten | 84 |
| Rhenium  | 15 |
| Yttrium  | 1  |

#### EXAMPLE 12

|          |    |
|----------|----|
| Tungsten | 79 |
| Rhenium  | 20 |
| Yttrium  | 1  |

Results similar to those of Example 1 were obtained with each of these alloys exhibiting room temperature ductility and fabricability.

The invention in its broader aspects is not limited to the specific details shown and described but departures may be made from such details within the scope of the accompanying claims without departing from the principles of the invention and without sacrificing its chief advantages.

What is claimed is:

1. A ductile high-temperature alloy consisting essentially of tungsten as the principal component, from 3 to 20% by weight of rhenium, and from .05 to 3% by weight of a metal additive selected from the group consisting of yttrium and mixtures of yttrium and cerium.

2. A ductile high-temperature alloy consisting essentially of tungsten as the principal component, from 5 to 15% by weight of rhenium, and from .05 to 3% by weight of a metal additive selected from the group consisting of yttrium and mixtures of yttrium and cerium.

3. A ductile high-temperature alloy consisting essentially of tungsten as the principal component, from 3 to 20% by weight of rhenium, and from .05 to 3% by weight of yttrium.

4. A ductile high-temperature alloy consisting essentially of tungsten as the principal component, from 3 to 20% by weight of rhenium, and from .05 to 3% by weight of a mixture of yttrium and cerium, the ratio by weight of yttrium to cerium being from 1:2 to 2:1.

5. A ductile high-temperature alloy consisting essentially of tungsten as the principal component, from 3 to 20% by weight of rhenium, and from .05 to 3% by weight of a mixture of yttrium and cerium.

6. A ductile high-temperature alloy consisting essentially of tungsten as the principal component, from 5 to 15% by weight of rhenium, and from .05 to 3% by weight of yttrium.

7. A ductile high-temperature alloy consisting essentially of tungsten as the principal component, from 5 to 15% by weight of rhenium, and from .05 to 3% by weight of a mixture of yttrium and cerium.

8. A ductile high-temperature alloy consisting essentially of tungsten as the principal component, from 5 to 15% by weight of rhenium, and from .05 to 3% by weight of a mixture of yttrium and cerium, the ratio by weight of yttrium to cerium being from 1:2 to 2:1.

9. The process of producing a ductile high-temperature tungsten-base alloy comprising the steps of: compacting a mixture of finely divided powders consisting essentially of from 3 to 20% by weight of rhenium, .05 to 3% by weight of a metal additive selected from the group consisting of yttrium and mixtures of yttrium and cerium, and the balance tungsten, heating the resultant compact in a hydrogen atmosphere at a temperature of from 1400 to 2700° F. for a time period sufficient to achieve outgassing of a substantial portion of occluded and adsorbed gases and vapor phase compounds of oxygen and nitrogen with yttrium and cerium and to impart a density of from 55 to 75% in the compact, sintering the compact in a dynamic vacuum at a temperature of from 3600 to 4200° F. for a time period sufficient to achieve from 85 to 98% density in the compact, whereby a ductile tungsten-base alloy having high strength at high temperatures and fabricability at low to moderate temperatures is created.

10. The process of claim 9, in which the compact is heated in a hydrogen atmosphere to a temperature of about 2200° F. for 2 hours.

5 11. The invention as defined in claim 9, in which the compact is sintered in a dynamic vacuum at a temperature of about 4000° F. for from 1 to 4 hours.

#### References Cited

##### UNITED STATES PATENTS

10 3,138,453 6/1964 Foster et al. ----- 75—176X

##### FOREIGN PATENTS

816,135 7/1959 Great Britain ----- 75—176

15 BENJAMIN R. PADGETT, Primary Examiner

R. L. TATE, Assistant Examiner

U.S. CL. X.R.

75—221, 225